

Patented Mar. 12, 1929.

1,705,088

# UNITED STATES PATENT OFFICE.

PERCY A. HIPPLE, OF ATLANTA, GEORGIA.

## METHOD OF LAYING CONCRETE PAVEMENTS.

No Drawing.

Application filed October 7, 1927. Serial No. 224,773.

This invention relates to an improved process of producing concrete pavement slabs and particularly to the process of finishing the wear surface of such slabs.

5 Primarily, the invention seeks to produce a concrete paving slab having a surface of high wear resistant properties, such surface of the finished slab being of a substantially non-porous character, due to the fact that pores 10 which normally occur in the surface of the slab, when formed according to present day methods, are filled with fine solid particles by the finishing step of the present invention.

In substantially all commercial processes 15 of placing and finishing concrete slabs, the compacting and working of the slab to a high degree of uniformity and surface finish removes only a minor portion of the water present in the concrete mix for hydration of 20 the cement, the major portion of such water being retained in the mass by the capillary attraction of the concrete aggregate.

Agitation effected by the compacting and 25 finishing of the slab having ceased, the retained water is slowly released by the settling of the finer particles in the concrete mass, these fine particles coming to rest one against the other and having a tendency to free the water and force it to the surface of the slab.

30 When enough water is released from the lower portion of the slab to saturate the upper portion of the concrete mass, a surface tension is created and all the remaining surplus water is quickly drawn to the surface. This accounts 35 for the water sheen or water film on concrete surfaces, which may be observed immediately before the initial setting of the cement. However, the water sheen is dissipated rather quickly by evaporation until the surface tension is broken, at which time the remaining 40 moisture on the surface is drawn by capillary attraction back into the interior of the slab and immediately thereafter the initial setting of the cement begins.

45 In the production of the slabs, the close interrelation of the aggregate particles is essential to the production of a slab of desired strength, and this association of said particles is effected by the various means which are used 50 for leveling the concrete mass to the desired contour and elevation. The various finishing processes utilized in connection with the production of the slabs all also tend to work the concrete into a compact mass, so as to better 55 effect this close association of the particles which is dependent upon the removal of the

water and entrapped air in the concrete mass. The appearance of the water film at the surface of the concrete slab, as previously mentioned, not only prevents this interlocking 60 and settling together of the fine cement particles at the surface in the manner in which such particles become associated lower down in the structure and which is necessary to the attainment of maximum density and strength, 65 but, on the contrary, the water coming to the surface of the slab actually forces the particles at the surface upward and apart, thereby creating pores and capillaries in the act of passing outward. As a result, the subsequent 70 quick dissipation of the water film or sheen leaves the surface of the finished concrete slab in a disturbed porous state, much below the natural strength developed by the material under ideal conditions. 75

The porosity of the surface of the concrete pavements laid as above described, causes such pavements to be highly absorbent of moisture and subject to constant expansion stresses, a disturbing factor in all present day 80 concrete paving construction. Furthermore, the disturbed porous state of the cement particles near the surface decreases the strength and resistance of such surface against the wear and tear of traffic and other agencies of 85 destruction.

In order to prevent the formation of a wear surface of such porous characteristics, the present invention contemplates a method of finishing the surface of a concrete pavement 90 slab wherein the pores produced on the surface during the accumulation of the water at such surface will be filled with finely divided particles of some suitable substance which does not have any detrimental effect on the 95 slab. More specifically, this finishing process consists in directing a fluid spray against the surface of the slab, whereby solid particles present in the water covered surface will be forcibly driven into the pores in the slab surface. In carrying out the present method, the finely divided solid particles may be in the form of the cement particles which are forced upward and apart by the water rising to the surface of the slab, although, if it is desired, 100 additional particles of cement may be distributed over the slab surface or other solids, such as stone, dust, or sand, may be superficially applied on the surface being finished. For forcing the particles into the pores a 110 preferably water spray or other fluid spray not chemically deterrent to the setting of the

concrete may be used or air may be utilized, it only being necessary that a spray of sufficient force be applied to the surface being finished, so as to force into the pores the cement particles in the water sheen or the cement particles or other solids previously applied to the surface. It will be understood, of course, that the spray used is very fine and the amount of liquid used is not sufficient to in any way damage the surface of the cement by washing out any of the cement or fine sand.

Specimens of concrete slabs have been produced in accordance with the present invention, as follows: A batch of concrete in proportion 15 portion 1 part cement, 2 parts sand and 4 parts washed gravel (a mixture which is the standard for highway pavements laid down by the Federal Bureau of Roads) was placed in forms, compacted and finished as nearly as 20 possible in the manner in which the average pavement slab is finished today. After water, which was forced out in the process of finishing, had drained, the water sheen or film appeared on the surface of the slab and, the 25 surface of the slab immediately subjected to a fine spray of water similar in fineness and density to the liquid spray delivered from the nozzle of an ordinary paint spray. It could be observed that the downward force of this 30 spray of water caused the cement particles in the surface of the slab to settle close together and close all the pores. When it was apparent to the naked eye that all pores had been closed and that the spray had no further effect on 35 the cement surface, the spray was discontinued and the specimen considered finished.

Where additional cement particles or other solids were applied to the surface of the slab, the concrete mix was placed in a form and 40 preliminarily finished, as described in the previous example. However, immediately upon the appearance of the water sheen or film, the surface of the slab was subjected to a blast of neat cement delivered from above 45 by means of an instrument similar to a sand blaster. It could be observed that this cement blast was closing the pores created in the surface of the slab, by the upward movement of the water sheen, and such cement blast could 50 be plainly seen to exert a settling influence on the wet surface. The cement spray was continued until the surface was apparently uniformly or evenly coated with neat cement, whereupon the water spray described in the 55 preceding example was immediately applied. The water spray was continued until it was apparent to the naked eye that all the pores were closed and all of the superficially applied neat cement tightly packed. At this 60 time the water spray would have no further effect on the cement surface, so that the spray was discontinued and the slab considered finished.

While water has been specifically mentioned in the examples given, it is believed

that in lieu thereof any liquid not chemically deterrent to the setting of the cement may be used for the spray and would effectively achieve objects sought by the present invention. Instead of a liquid, an air blast alone 70 would probably suffice, as any agency that will agitate the concrete surface at the time of the appearance of the water film will improve the texture of the surface. Undoubtedly, the air blast would accelerate the surface 75 tension at the time of the water sheen and would more quickly draw off the water, and, once the surface tension is broken under the air blast, said blast would have a direct effect on the cement particles in the surface, tending 80 to drive such free particles into the pores formed in the slab.

Slabs produced in accordance with the present invention have been found by actual tests to have exceedingly high wearing properties. A sample of a slab made in accordance with the ordinary practices of today; a second slab made by the use of the water spray alone; and a third slab made by the use of the superficially applied neat cement and water 90 spray were all furnished to one of the State schools of technology at whose highway material laboratory the same were subjected to wear tests. For the purposes of these tests the surfaces of the several blocks were ground 95 with carborundum stones, corresponding to about two years' wear on a medium traffic street. Below is given a table showing the cubic inches worn off per square foot of surface and the wear in per cent of a 6 inch pavement. As the three specimens appear in the table in the order in which they are above listed, it will be observed that both of the samples made in accordance with the present invention possessed much higher wearing 100 properties than the ordinary slab, the slab made by the use of superficially applied cement and water spray possessing wearing qualities about six times as great as the ordinary slab.

|                                            | Specimen 1. | Specimen 2. | Specimen 3. |
|--------------------------------------------|-------------|-------------|-------------|
| Cu. inches worn off per sq. ft. of surface | 6.95        | 1.87        | 1.15        |
| Wear in per cent of a 6" pavement          | 0.7%        | 0.22%       | 0.13%       |

#### What I claim is:

1. The process of producing concrete pavement slabs which consists in permitting water used in the concrete mass to hydrate the cement to accumulate in film like form on the surface of said slab and subsequently forcing particles of cement carried in said water film into pores formed in said surface during the accumulation of said water film by means of a fluid spray such as water.

2. The process of finishing the wear surfaces of concrete slabs, which consists in directing a blast of fluid against said surface to

forcibly introduce free solid particles into pores formed in said surfaces by exuding water initially used in the concrete mix for hydrating the cement therein.

- 5 3. The process of finishing the wear surfaces of concrete slabs, which consists in permitting the formation of a water sheen or film on the surface of the slab, then applying a coating of finely divided solids to the slab 10 surface, and finally forcing the solids into pores formed in said surface during the formation of said water sheen by a fluid spray of extreme fineness and of a volume insufficient to wash the solids out of the pores.
- 15 4. The process of finishing the wearing surface of a concrete slab which consists in permitting the accumulation of a water sheen or film on said surface, then depositing finely divided particles of a solid on said surface, 20 and then spraying said surface with a fluid to force said particles in pores formed in said surface during the accumulation of said water sheen, said spray being of a fineness and

volume insufficient to wash out the solids from the pores. 25

5. The process of finishing the wearing surface of a concrete slab which consists in permitting the accumulation of a water sheen or film on said surface, then depositing fine particles of neat cement on said surface, and 30 finally spraying said surface with water to force the neat cement into pores formed in said surface during accumulation of said water sheen, said spray being of a degree of fineness and of a volume insufficient to wash 35 the neat cement from the pores.

6. The step in finishing concrete pavement slabs which consist in forcibly introducing fine particles of cement into the pores formed in the surface of said slabs by the rising water mixed with the mass of concrete for hydration of the cement therein, by directing 40 against the surface of the pavement slab a fine spray of a fluid not chemically deterrent to the setting of the concrete.

PERCY A. HIPPLE.